

Sept. 30, 1924.

1,510,173

M. HOSENFIELD

MANGANESE PEROXIDE ANOD.

Original Filed Sept. 14, 1923

FIG. 1



FIG. 2



FIG. 3



FIG. 4



by Knight Bros  
J. C. H. & Son

## UNITED STATES PATENT OFFICE.

MARTIN HOSENFIELD, OF BERLIN-CHARLOTTENBURG, GERMANY, ASSIGNEE TO SIEMENS & HALSKE, AKTIENGESELLSCHAFT, OF SIEMENSSTADT, NEAR BERLIN, GERMANY, A CORPORATION OF GERMANY.

## MANGANESE-PEROXIDE ANODE.

Original application filed September 14, 1923, Serial No. 662,754. Divided and this application filed May 1, 1924. Serial No. 710,311.

To all whom it may concern:

Be it known that I, MARTIN HOSENFIELD, a citizen of the German Empire, residing at Berlin-Charlottenburg, Germany, have invented certain new and useful Improvements in Manganese-Peroxide Anodes, of which the following is a specification.

My invention relates to improvements in manganese peroxide anodes which are made according to the process forming the subject matter of my copending patent application Ser. No. 662,754 filed on 14th September, 1923. The invention consists in the anode itself as a new article of manufacture.

In the drawing two different examples of the new anode are given. Fig. 1 shows one construction in side elevation and Fig. 2 in a vertical section. The Figs. 3 and 4 show the upper part of the other example also in elevation and vertical section.

The improved anode consists of a carrier plate 1 which determines the shape of the finished anode and consists of a substance which is in regard to the object in view chemically and also electro-chemically indifferent. To this carrier the manganese peroxide is applied in such a manner that a coating on the surface of the carrier is produced. This coating can penetrate into the carrier in such a manner that it is saturated with the manganese peroxide. In this event also the peroxide will form a dense coating on the surface of the carrier. Fig. 2 shows a carrier 1 of porous material, for example infusorial earth, which has been saturated with manganese nitrate and then burnt at a temperature over 100°. The granulous material of the anode has been filled by the manganese nitrate which is decomposed in the burning process and converted into the manganese peroxide. Near the surface of the carrier the peroxide forms a dense coating 2 on the carrier.

As shown in Fig. 4 the surface of the carrier is roughened at 3 for the purpose of better securing the manganese peroxide.

Before applying the coating of the manganese nitrate to the carrier it may be mixed with pure amorphous manganese ore and the carrier can be saturated or pasted with this mixture. The amorphous manganese

ore is then a good and cheap substitute for a part of the expensive crystalline manganese peroxide.

The conductivity of the manganese peroxide anode may be improved as well known by an electrolytically produced coating of lead peroxide. This coating 4 is shown in Fig. 2.

The contact carrying the current to the anode consists of a piece 5 of carbon or graphite which receives the upper end 6 of the carrier in a groove 7. The lower edges of the sides of the contact piece are provided with teeth 8 meshing with corresponding teeth along the upper edges of the carrier 1 which is somewhat enlarged at this part. Into the side parts of the contact 5 and the upper part 6 of the carrier bolts 9 of carbon are inserted. When saturating or impregnating the carrier in the inverted vertical position with the manganese nitrate or when applying the paste and burning the carrier in this position a small portion of the nitrate flows between the contacting surfaces of the contact piece and the carrier and makes a very good contact between them. The coating of lead peroxide 4 is also passed over the point of junction between the carrier and the contact piece 5. In this manner an intermediate resistance to the passage of the electric current is effectively avoided.

After the carrier has been united with the contact piece 5 by burning side pieces 10 of paraffinated carbon are fixed to the contact piece by metal plates 11 and screw bolts 12. These paraffinated pieces 10 are provided for the purpose of preventing the electrolyte from ascending to the metal parts.

What I claim as my invention and desire to secure by Letters Patent is:—

1. Anode of manganese peroxide for electrolytic purposes, comprising a carrier for the peroxide having the shape of the anode and consisting of a substance which in regard to the object in view is chemically indifferent.

2. Anode of the type described, consisting of a carrier in shape of the anode having a dense coating of manganese peroxide.

3. Anode of the type described, consisting of a carrier in the shape of the anode hav-

ing a dense coating of manganese peroxide, and means to secure said coating on the surface of the carrier.

4. Anode of the type described, consisting of a carrier in the shape of the anode made of porous material, the cavities of which are filled with manganese peroxide.

5. Anode of the type described, consisting of a carrier of infusorial earth in the shape of the anode, the cavities of which are filled with manganese peroxide.

6. Anode of the type described, consisting of a carrier in the shape of the anode having a dense coating of manganese peroxide and a contact piece of carbon.

7. Anode of the type described, consisting of a carrier of porous material the cavities of which are filled with manganese peroxide having a dense coating of manganese peroxide and a contact piece of carbon.

8. Anode of the type described, consisting of a carrier of porous material in the shape of the anode, the cavities of which are filled with manganese peroxide, having a dense coating of manganese peroxide and a contact piece of carbon at its top, wherein all the cavities between the carrier and the contact piece are filled with manganese peroxide.

30 9. Anode of the type described, consisting of a carrier in the shape of the anode made

of porous material with a roughened surface, manganese peroxide filling all the cavities of the carrier, and means arranged at the top of the carrier for conducting the current to the anode.

10. Anode of the type described, consisting of a carrier in the shape of the anode, manganese peroxide applied to the carrier, a contact piece arranged at the top of said carrier for conducting the current to the anode, metallic means for holding the anode, and pieces of paraffinated carbon arranged between said contact piece and said metallic means.

11. Anode of manganese peroxide for electrolytic purposes, comprising a carrier for the peroxide having the shape of the anode and consisting of a substance, which in regard to the object in view is chemically indifferent, and a coating of lead peroxide.

12. Anode of the type described, consisting of a carrier of porous material, manganese peroxide filling all the cavities and coating the surface of the carrier, a contact piece for conducting the current to the anode, and a coating of lead peroxide upon the carrier as well as the point of junction between it and the contact piece.

In testimony whereof I affix my signature.

MARTIN HOSENFIELD.